

## UNITED STATES PATENT OFFICE

2,406,097

METHOD FOR PRODUCING WHITE  
SODIUM ROSINATES

Avery A. Morton, Watertown, Mass.

No Drawing. Application January 21, 1942,  
Serial No. 427,679

8 Claims. (Cl. 260—105)

## 1

This invention relates to sodium rosinates and method for producing the same.

More particularly it relates to the producing and isolating of alkali metal rosinates which have the peculiar characteristics that they are white, and also that they are free from certain objectionable features hitherto considered typical of rosinates.

The invention is herein illustratively described with reference to its bearing on the soap industry, because of its promoting rosin to the status of having a market and cooperative utility among materials for making first class soap. The high value of the rosinate of the invention in this respect comes from the fact that it enables white soap to have the advantages which attend the use of rosin, and yet be free from defects and disabilities, hitherto considered inseparable, which have excluded rosin from soap of that class. But the utility is not limited to soap. Many or all industries using rosinates or rosin may benefit; and with the aid of this invention the introduction of rosin products into still other fields may be expected.

Hitherto rosin has depreciated soap by imparting to it a disapproved characteristic yellowish brown color. Bars of white soap embodying the white rosinate of the invention have been found not losing their whiteness as they age under ordinary conditions of air, moisture and daylight. And there are improvements in other respects over rosin as heretofore used.

I have demonstrated that from the "sodium rosinate" of ordinary use there can be produced two distinguishable substances, both of which are rosinates. As hitherto known these are so thoroughly intermingled, are so much alike, and in mixture, are so dominated by the character of one of them that the benefits of the other of them have not before been available or even known, so far as I am aware. Whatever the chemical distinction that may ultimately be found between these two, the present specification discloses a way of producing them separately from the customary "rosinate." It is sufficiently distinctive for purposes hereof to designate these respectively "dark rosinate" and "white rosinate." My discovery of the white rosinate, and of a way to segregate it, contributes to industry rosinates of sodium or other alkali that appear to be indus-

## 2

trially useful for all purposes for which the customary rosinates heretofore known can be applied, lacking no useful function by reason of the absence of the dark rosinate, but being free from the burdens hitherto attending rosinates. The process of segregation includes a step which utilizes the preferential affinity of a rosin solution for the dark rosinate. The dark rosinate, and resenes and esters, can be separately recovered, for uses to which they are appropriate.

The closest approaches of prior art, known to me, are found among methods proposed for lightening the color of rosin or rosinates, but none of those, nor any of those which separate the rosin into components, or crystallize it as abietic acid, has resulted in furnishing white rosinate for the soap maker. This is so universally recognized that the expressions "rosin soap" and "yellow soap" are practically synonymous.

Among these prior proposals, that shown in United States Patents Nos. 2,085,151 and 2,085,152 issued to Georgi would treat a solution of abietic acid or resin, preferably a ten per cent solution, in a solvent which is a non-solvent of the alkali and of the abietate, with alkali "sufficient to substantially neutralize the abietic acid present." The product of this treatment is stated to be "alkali abietate in rather pure form; that is, free from resenes or the like," and these patents also say their product is "substantially free from color bodies"; but tests show that color bodies are present in appreciable quantity. The patent to Kesler No. 1,633,764 proposed to precipitate the alkali acid salt while allowing the resenes to remain in solution, to make a product which does not become moist and sticky, and from which is obtainable "abietic acid free of impurities." However, it removes only the resenes and whatever of the color bodies are present in the resenes. The product still contains the colored salts of rosin acids. In the process of French No. 2,012,125 for highly purifying rosin, an aqueous petroleum suspension of rosinate is dehydrated by hot petroleum so that the alkali rosinate separates from the solution. The "crystals of the new product" are, according to the patent, "readily amenable to washing or other purification treatment." The product obviously was not white.

None of these methods for improving the color makes a rosinate usable in white soap. Mere re-

moval of the resenes and such color bodies as are part of the resenes, i. e. unsaponifiable matter, is not sufficient.

The inherent inability of prior procedures to separate white rosinates from dark is perhaps the reason why white rosinate has, so far as I am aware, remained unknown until my discovery.

The discovery has shown further that the objectionable features of rosin in soap are not associated with all rosinates, but are more particularly attributes of the substances which the invention eliminates. I show that there is a difference of solubility, as well as of color, between the dark and the light; and further that all of the substances having offensive color characteristics, normally found in the mix after treating rosin with a base, can be held, preferentially over the white rosinates, in a solution herein described. The described procedure is successful without needing an exact theory as to how or why this is so.

To understand my attainment of a product having the whiteness which is demanded in soaps of high quality one may bear in mind the fact that rosin contains some oxidized or colored acids; that salts of those acids are dark; that the process herein to be disclosed applies the principle of preferential solubility, by proportions, controls and adjustments, so as to separate those dark salts from other salts which are white; and that the ordinary sodium rosinate, hitherto a soap material of low esteem, always possesses these unwanted characteristics because there is always some of the dark rosinate present in it, however highly purified or "light colored" it may be.

The process comprises a treating of rosin with a base, and a separating of the product into two parts, one of which has the white sodium rosinates. The other part is a solution containing all of the colored substances, including dark sodium rosinates, resenes, rosin esters, and some unneutralized rosin. This solution is amenable to further separation if desired. The preferential solubility of the dark substances depends upon the solution holding also a sufficient concentration of rosin. The greater the concentration of rosin in the solution, the more surely will the dark rosinates be held in solution.

For greatest economic efficiency, the quantity of solvent and the concentration of rosin therein must be selected or adjusted so that the rosinate-dissolving capacity, made by the concentration of rosin, is sufficient to take up all of the dark rosinates, in addition to the resenes, esters and other colored components; and yet is limited so that the solution will become saturated when all of those have been taken up, so that no considerable quantity of the white rosinates will be taken up. This saturated condition is what should be prevailing at the stage when the white rosinates are being separated from the solution. Before that stage the concentration of rosin present will preferably be great enough so that it can undergo diminution with the progress of the reaction, and yet be correct in amount to produce the desired saturation, at the time and temperature of filtration.

To demonstrate the theory which underlies this invention one may observe that dry sodium rosinate is insoluble in kerosene. If, however, rosin in sufficient quantity is added to the kerosene the sodium rosinate both white and dark will dissolve. If, on the other hand, rosin is present in insufficient quantity, i. e. if more ros-

inate is present than can be dissolved with the given amount of rosin, the dark rosinate will be taken and held preferentially, leaving more or less of white rosinates in a solid form which can be recovered by filtration. As an illustration of this theory, 40 g. of a powdered dry sodium rosinate, made from WG rosin and therefore containing a quantity of dark sodium rosinate, can be added to 190 cc. of kerosene, and the mixture heated to 140° C. with stirring, without there being any appreciable dissolving of the rosinate. However, upon adding 40 g. of rosin, and repeating the process of heating and stirring over a period of two hours, most of the rosinate becomes dissolved. When the whole process is repeated using 80 g. instead of 40 g. of dried sodium rosinate a large portion of the rosinate remains undissolved. When recovered by filtration this material is found to be white.

Another method for demonstrating the theory which underlies this invention is to add a limited quantity of sodium carbonate to a petroleum solution of rosin. As the carbonate reacts with the rosin and forms sodium rosinate, the latter goes into solution. The addition and reaction of more and more carbonate eventually produces more rosinate than the solution can hold. The white sodium rosinate then comes out of solution as a precipitate and the dark colored rosinate is held preferentially. By adjusting empirically the quantities of alkali, rosin and hydrocarbon solvent it is possible to produce a highly desirable condition for operation of the process. As a specific illustration of this second method of showing the solubility of sodium rosinate in a petroleum solution containing rosin, and also as a demonstration of one method of practicing this invention, three cases are here given: First, (a) use of alkali in what may, for this purpose, be called a "low" ratio of alkali makes sodium rosinate that will remain in solution, because of the solubility of all sodium rosinates in a solvent which also holds unneutralized rosin in solution. It is assumed in each of these illustrations that the process is run as long as the sodium rosinate continues to be formed at a reasonable rate. Second, (b) what may be called a "moderate" ratio of alkali makes more sodium rosinate, than the solution can hold; the fraction that precipitates out is a white rosinate; and whatever dark rosinate is present continues in solution. But (c) with a ratio of alkali so "large" that most of the rosin acids becomes neutralized, the power of the solvent to hold the dark sodium rosinate drops sharply, and the precipitate is a mixture of the white and dark sodium rosinate, and therefore is not white. Thus, by selecting the proportion of alkali which is introduced for the reaction, whiteness of precipitate can be obtained, care being taken that the concentration of rosin does not become too much reduced.

Quantitative examples illustrative of the foregoing cases follow:

(a) The addition at 110° C., with stirring, of 40 g. of anhydrous sodium carbonate to a solution of 480 g. of WG rosin, dissolved in enough kerosene to make a total volume of approximately 1750 cc., which makes the concentration of rosin be about 36% in the total weight of solution, if the kerosene has a specific gravity of 0.73, causes the described reaction, which can proceed to a conclusion in about one and one-half hours without the temperature having risen above 133° C. However, the sodium salt which has been produced remains largely dissolved in the reaction

mixture, even when the kerosene solution is allowed to cool to room temperature.

In case (b), where the ratio of carbonate to rosin is, say 2 to 12 instead of 1 to 12, and the heating and stirring is carried out until reaction has been effected at a final temperature of 145° C., a precipitate is produced which is white or so near to white that, after separation from the solution and from adhering liquid, it is suitable for use in white soap, or for use as a high quality of size for paper, or for any use for which a white sodium rosinate may be desired.

But (c) when the ratio of carbonate to rosin is made 3 to 12 the color of the precipitate has been found to fall into the range of grayish white or tan. If a still higher proportion of alkali is used the color becomes brown.

The foregoing examples respectively show, first, all sodium rosinates caused to dissolve in a hydrocarbon solvent by the presence of rosin; second, dark rosinate kept in the solution preferentially, while the precipitate is entirely white rosinate; and, third, dark rosinates precipitated to some extent when there comes to be still less rosin present in the solution. These also show that practice of this invention may require adjustment of a number of factors.

The principal variables in the process are, (A) concentration of rosin in the solvent, which is best kept as high as possible, for it diminishes continuously throughout a reaction in which rosinate is being produced, and yet should at the end of reaction be such that the colored rosinate and all other coloring matter is surely held in solution in the mother liquor; (B) adjustment of the ratio of alkali present for the reaction; (C) selective control of the temperature, which must be high enough to effect reaction, and at times high enough to increase the solubility so as to prevent precipitation of dark rosinate, but preferably will be held to moderate limits, in order that cracking of the rosin acids shall be avoided; (D) suitable agitation, the more vigorous the better, to make good contact between the solid alkali and the rosin acids, and to promote prompt escape of all volatile products; (E) adjustment as to the duration time, since the rosinate first precipitated will be white, but that precipitated later may be dark, as when the process goes to completion, and the reduction of concentration of the rosin in the solution, and the current conditions as to quantity of alkali, temperature or other factor may be, or may come to be, such that toward the end dark bodies are precipitated; (F) preferably, that the source material chosen should be cleaned crude gum, or else be light colored rosin; and (G) for the best commercial success, that the solvent and the alkali be of inexpensive kinds, for which at present kerosene and sodium carbonate are satisfactory.

The invention can be practiced with wide variation of these conditions. Herein will first be given observations pertaining when there is a relatively high concentration of rosin, which might be called a preferred region for operating the process. In this the above mentioned variables can be changed within wide limits without greatly affecting the result. Second, the case will be stated where the conditions are in a region which can be described as critical, in that the factors are so inter-dependent that if any one of them varies too far from its normal or advisable value the control or adjustment of others becomes very important. The conditions for successful operation will be illustrated; in addition to which

it should be understood that the pre-determination of the adjustment of factors to be used in any practicing of the process industrially can, if necessary, always be approached empirically by allowing sodium carbonate or other suitable alkali to react with rosin, in a solvent having a high concentration of rosin, and the progress of reaction with precipitation of sodium rosinate be observed until the obtainable quantity of white sodium rosinate has been formed, and adjustments made of rosin concentration, alkali, temperature, and duration as may be desired.

The proportion of rosin in the solvent is the most important of the factors mentioned above; for if the initial concentration of rosin is sufficiently high the concentration existing at the end of the reaction will not have fallen so low as to fail to hold in solution the undesired rosinate and the other undesired substances. Although the having of the concentration adequate at the time of separation of the white rosinate is of ultimate importance, it is most practical and informative to state the concentration of rosin in terms of the amount at the beginning of reaction, as is done in the examples here given.

However, in any instance, the concentration of rosin existing at the time of filtration can be found by analysis. Concentrations so found in a series of trial operations on samples can be used as a guide to select the initial concentration to be employed in a main operation on any particular lot of rosin. In various lots the contents of dark rosinate may differ. If it is desired to attain the highest practicable yield of white rosinate, with a minimum of attendant costs, the concentration of rosin for dealing with any particular lot should be such as will make the saturation point for rosinates occur when all of the dark rosinate has been dissolved, and approximately all of the white rosinate remains undissolved. By a series of laboratory tests applying the process to samples from a particular lot with diminishing concentrations of rosin, in successive samples until one is found whose isolated rosinate product is not white, it can be learned which initial rosin concentration value will be commensurate with a rosinate-dissolving capacity of the rosin solution that is limited so that the solution becomes saturated with rosinate coincidently with the completion of the dissolving of all dark rosinate that exists in the particular lot to be treated, or that is produced from it. In that case the rosinate will have been fractioned so that the undissolved rosinate will be all of the white rosinate that is available, a modicum being already dissolved.

An analysis may be made by shaking the filtrate of the sample operation, viz, the mother liquor which has passed through the filter, with water to take out sodium rosinate equivalent to what was in solution at the time of filtering; then extracting the rosin therefrom with sodium carbonate; and after that distilling away the mother liquor to recover resenes and esters. This series of operations provides data by which concentration of combined and uncombined rosin acids and of other constituents may be calculated. The quantity of solvent may be assumed not to have changed appreciably during the reaction; but if any is known to have been lost, or added, due allowance can be made. The weight of combined rosin is obtainable by acid treatment of the rosinates found in the residue and those found in the filtrate. The total of combined and uncombined rosin, plus the small amount of resenes and esters, found by this analysis, is comparable with

the various percentages of rosin mentioned in the tables which follow; and the optimum concentration of rosin required to be provided in the rosin solution, for the filtration step, in producing white rosinate from the particular lot of rosin thus sampled, can thus be known.

The best form of the process, in brief, involves the making of a non-aqueous mixture of alkali with an inert solvent holding in solution a very high concentration of rosin acids, although not too high for agitation to be effected, about 45 to 50% by weight if petroleum with a specific gravity of 0.73 is used; heating, stirring and maintaining fluidity in the thick mixture while reaction producing rosinate continues at restricted temperature; fractioning the solute by precipitating the white rosinate from solution while the mother liquor has sufficient concentration of rosin to retain in solution all rosinates and other substances having color; separating the precipitate from the solution by filtration; and, if desired, washing the separated matter clean of the mother liquor, to make the final product. Details will appear hereinafter of steps and restrictions that may be applied for controlling the source material, the solution and the fluidity of the mixture, the reaction, and the fractioning of the solute. These may vary considerably, relative to each other, while still giving an optimum of whiteness. Also they may vary among themselves according to the grade of final product which is wanted, in case it is adjudged admissible that the extremely white be slightly shaded by containing a modicum of lower grade mixed with it, for lower cost or greater yield.

The term "rosin" as used herein may be considered to include any material whose acid component has the composition of approximately  $C_{20}H_{30}O_2$ .

In Table I are illustrative examples in which, at the beginning, rosin was concentrated in kerosene in the high ratio of about 1 g. of rosin to 1.1 g. of petroleum solvent, a concentration of about 50%. A result of this high concentration is that at the end of the process, notwithstanding the diminution of rosin which has occurred, the rosin concentration is still great enough to hold the color bodies in solution, even when the poorest grade of rosin is used, while the white sodium rosinate is precipitated. Formation of sodium rosinate and evolution of carbon dioxide and water begin at a temperature only a little above 100° C., according to the equation:



particularly if the mass starts to gel. The petroleum may advantageously contain some low boiling fraction, which by its own volatilization will facilitate the removal of the small amount of water that is formed by the neutralization of the rosin. Removal of this small amount of water helps to prevent gelling. A little additional petroleum may be added to compensate for any loss by volatilization, or to facilitate the stirring if the mixture becomes extremely thick. Stirring is continued while the mixture is held at 140° C. to 150° C. during the last hour, without the temperature rising materially above the limit indicated, until the reaction is substantially complete, as shown by cessation of escape of water or of carbon dioxide set free by the reaction. The mixture is then allowed to cool to about 120° C., where it is filtered to separate the precipitate, more of which comes out of solution as the mixture cools. Filtration can be carried out at 90° or even lower but the mixture is correspondingly thicker and harder to filter. The precipitate is found to be snow white sodium rosinate. All color bodies, particularly the dark colored sodium rosinates, pass through the filter because the rosin is still sufficiently concentrated to hold them in solution in the mother liquor, in which the white sodium rosinate is relatively insoluble, so that it is retained by the filter. The filtration can be effected by any of the recognized varieties of apparatus, including the centrifuge.

The centrifuge will ordinarily leave the precipitate sufficiently clear of the mother liquor, but, if desired, the white precipitate may be washed with small quantities of kerosene or other petroleum, to remove the mother liquor from it, until the liquid coming away is colorless. Low boiling petroleum can be employed to remove higher boiling wash liquid; and the low boiling petroleum can be cleared away by promoting its evaporation.

If it is desired to separate the unreacted excess of alkali, that was retained by the filter with the rosinate, this can be cleared from the rosinate by dissolving them both in water and then salting out the rosinate, or in any other known manner. If the white rosinate is to be used in soap this step can be postponed and the result attained at the corresponding stage of the soap making.

The completing of filtration is considered to end the process of the invention, the white rosinate being then isolated from the dark rosinates. The free alkali that may be present with it is inconsequential. This would be some of the alkali that was introduced for the reaction but became covered by precipitated rosinate and thereby was prevented from reacting.

TABLE I

| No.    | Rosin,<br>g. | Grade        | Na <sub>2</sub> CO <sub>3</sub> ,<br>g. | Sol.<br>vol.,<br>cc. | Percent<br>alkali<br>to rosin,<br>percent | Concen-<br>tration of rosin<br>in solution,<br>percent by<br>wt. | Max.<br>temp.,<br>°C. | Time,<br>hrs. | Yield,<br>percent | Color       |
|--------|--------------|--------------|-----------------------------------------|----------------------|-------------------------------------------|------------------------------------------------------------------|-----------------------|---------------|-------------------|-------------|
| 1..... | 120          | WG.....      | 39                                      | 285                  | 32.5                                      | 49                                                               | 150                   | 2.5           | 80                | Snow white. |
| 2..... | 120          | WG.....      | 31                                      | 285                  | 25.9                                      | 49                                                               | 150                   | 2.5           | 80                | Do.         |
| 3..... | 120          | WG.....      | 48                                      | 280                  | 40                                        | 50                                                               | 150                   | 2.5           | 81                | Do.         |
| 4..... | 120          | K wood.....  | 31                                      | 285                  | 25.9                                      | 49                                                               | 150                   | 1.5           | 78                | Do.         |
| 5..... | 132          | FF wood..... | 35                                      | 285                  | .....                                     | .....                                                            | 152                   | 1.8           | 70                | Do.         |

Anhydrous sodium carbonate having been introduced into the solution of rosin in kerosene at or below 110° C., heating is continued so that in an hour the temperature has risen to about 140° C. The mixture usually becomes very thick, and stirring must be vigorous to maintain fluidity,

In Example 5 the rosin was first dissolved in 800 cc. of ligroin, filtered while cold, concentrated, and then diluted to a volume of 285 cc. by addition of kerosene. These operations removed colored material which was insoluble in petroleum and would have contaminated the product. The

exact percentages are not known, in this example, because the quantity of petroleum-insoluble material, which was separated before carrying out the process, reduced the actual weight of rosin used.

Similar operations using as source material crude gum, of a kind which would ordinarily produce WG rosin, give parallel results, as shown in Table II.

TABLE II

| No.    | Gum,<br>g. | Na <sub>2</sub> CO <sub>3</sub> ,<br>g. | Sol.<br>vol.,<br>cc. | Per cent<br>alkali<br>to rosin,<br>per cent | Rosin in<br>solution,<br>per cent by<br>weight | Max.<br>temp.,<br>°C. | Time,<br>hrs. | Yield,<br>percent | Color       |
|--------|------------|-----------------------------------------|----------------------|---------------------------------------------|------------------------------------------------|-----------------------|---------------|-------------------|-------------|
| 6----- | 156        | 31                                      | 285                  | 26                                          | 49                                             | 146                   | 2.5           | 80                | Snow white. |
| 7----- | 152        | 39                                      | 285                  | 33                                          | 50                                             | 150                   | 2.5           | 80                | Do.         |

As the crude gum source material was about four-fifths rosin and one-fifth turpentine, the concentration of rosin was calculated on the basis of 80% rosin content in the gum.

In the above examples, in Tables I and II, the source material ranged from crude gum through WG rosin to FF wood rosin. The rosinate product in each of these cases was snow white. That from the FF wood rosin was not so beautifully snow white as the others, yet even in this case the product, when dissolved in water and precipitated by addition of salt, gave a product which in soap would have been satisfactory.

These examples illustrate the merit of having high concentration of rosin in the solvent, the limit being reached only when the mixture becomes too thick to stir or filter. First, the colored material (the colored rosinates as well as the colored resenes) is thereby readily held in solution. Second, it is possible to obtain good yield of high quality material in a single operation without the necessity of recycling. Third, it renders unnecessary many details of manipulation which becomes advisable when the strength of certain of the variables lies in a more critical zone, as indicated hereinafter. And a fourth advantage is that very cheap grades of rosin, such as FF wood, can be employed.

If, as in the above examples of preferred practice, there is so much rosin in the solvent that its weight approaches or about equals the weight of the solvent, this may be considered normal in the sense that the process will work comfortably even though the quantity of alkali, the temperature, or the grade of rosin, or all of these, lie in zones which under other conditions might be considered not so good. But if the rosin is only about half as much as the solvent, by weight, or less, the conditions of alkali, temperature and grade require critical consideration and restriction, lest the sodium rosinate obtained fail of having the characteristic white, or near whiteness, of the invention, or be not free from unsaponifiable matter.

Practice of this invention in such a less concentrated solution is what was referred to herein before as having conditions in a critical zone. Considerable variation of some of these conditions can still be allowed but such factors as the quantity of alkali, the temperature of filtration, and the grade of rosin must be considered much more carefully than is the case with the very concentrated solutions. Observations follow as to adjustment of alkali, then of the temperature, and next of the grade of rosin to be selected as a source material.

If the process is to be practiced with need for

care as to the ratio of alkali to rosin, the making of adjustment of the ratio of alkali means that the quantity of alkali which will give the desired result should be determined empirically, and that the quantity used, in proportion to the other substances present, be limited accordingly. The second example above given of the theory underlying the process shows how the quantity of alkali can be adjusted empirically so that a prod-

uct of suitable whiteness is obtained. The sensitivity is caused by the danger that within the customary time period so much rosin will be removed, as rosinate, from the solution that the desired retention of the dark colored rosinate in solution may not be realized.

If some of the dark sodium rosinate ceases to be held in solution the temperature of reaction may be raised, in order to assure that the dark rosinate shall stay in solution. In these cases a drop in temperature to 110° C. or lower before filtration will cause precipitation of moss-like aggregates of dark sodium rosinate; and these contaminate the product so as to render it unsuitable for white soap. To increase the solubility of the dark rosinate the temperature of filtration must also be raised; and the filtration process itself must be as rapid as possible (for example, a filtration by centrifuging) in order to complete the separating before the dark rosinate will have begun to precipitate. The more the alkali becomes consumed, i. e. the further the progress toward neutralization of all rosin acids present, within the time allotted for reaction, the greater is the danger of precipitation of dark rosinate occurring, and the greater is the care required to avoid that during filtration.

When operations are within the critical zone the grade of rosin selected for the starting material is of considerable importance. Light colored rosins which contain a minimum of colored material are much better than the darker grades of rosin. One of the best grades for production of white rosinate is crude gum, because of the smallness of the proportion of colored acids present.

The tabular showings of test examples which follow illustrate the varying effects obtained with the differing relations of materials, proportions, temperatures, kinds, etc., therein shown.

In Table III, the color of the rosinate obtained, ranging from snow white to tan, in all cases was better than the sodium rosinate prepared by conventional methods. The temperature at which sodium rosinate was recovered by filtration was below 110° C. for the better grades of product. Where the yield was high, however, higher temperatures were employed, even up to 160° in order to reduce precipitation of dark sodium rosinate which is apt to occur at this concentration of rosin in the solution. The temperatures indicate the maximum, and were those reached about an hour before the end of the reaction. The reaction sets in at about 107° C. although the carbonate was often added at much lower temperatures, for example, at 90° C. or even 80° C. Agitation was continued as the temperature rose

steadily. Although the final temperature is rather high in some of the experiments, the presence of alkali reduces the tendency for the rosin to decompose by cracking.

The various tables show that, at these low concentrations of rosin in kerosene, the yield of white rosinates is less. In general, they show that the better results attend the greater ratios of excess rosin in solution, the lower ratios of carbonate to rosin, the lower temperatures, and the shorter reaction times. However, in all cases, dark colored sodium rosinates have been removed, as can be shown by retrieving the remaining acids as the sodium salts and comparing their color with that of the material separated in the process.

TABLE III  
WG rosin and  $Na_2CO_3$  in kerosene

| No. | Rosin, g. | $Na_2CO_3$ , g. | Total mix, cc. | Concentration of rosin by weight in solution, percent | Ratio alkali to rosin, percent | Max. temp., °C. | Time, hrs. | Yield, percent | Sodium rosinate, color |
|-----|-----------|-----------------|----------------|-------------------------------------------------------|--------------------------------|-----------------|------------|----------------|------------------------|
| 8   | 525       | 90              | 1,750          | 36                                                    | 17.1                           | 156             | 2.25       | 47             | Snow white.            |
| 9   | 480       | 85              | 1,750          | 34                                                    | 17.7                           | 159             | 2.25       | 47             | Do.                    |
| 10  | 305       | 78              | 1,750          | 22                                                    | 25.6                           | 172             | 2.6        | 60             | White.                 |
| 11  | 300       | 75              | 1,750          | 22                                                    | 25                             | 182             | 2          | 59             | Gray white.            |
| 12  | 305       | 80              | 1,750          | 22                                                    | 26.2                           | 179             | 4.25       | 62             | Do.                    |
| 13  | 302       | 80              | 1,750          | 22                                                    | 26.5                           | 189             | 3          | 69             | Do.                    |
| 14  | 302       | 80              | 1,750          | 22                                                    | 26.5                           | 176             | 3          | 74             | Do.                    |
| 15  | 200       | 54              | 1,750          | 15                                                    | 27                             | 185             | 2.25       | 73             | Shady white.           |
| 16  | 302       | 90              | 1,750          | 22                                                    | 30                             | 179             | 3.4        | 75             | Do.                    |
| 17  | 302       | 100             | 1,750          | 22                                                    | 33.1                           | 184             | 3          | 79             | Cream white.           |
| 18  | 300       | 100             | 1,750          | 22                                                    | 33.3                           | 182             | 2.25       | 82             | Light tan.             |
| 19  | 400       | 160             | 1,750          | 28                                                    | 40                             | 192             | 3          | 82             | Tan.                   |

In computing the concentrations of rosin the specific gravity of kerosene is taken as 0.73.

In Nos. 8 and 9 low ratios of alkali to rosin are seen to go with snow white rosinate.

In Nos. 10-19 higher ratios of alkali to rosin, higher temperatures, and longer times of reaction, are seen to go with reduced perfection of whiteness, i. e., less complete separation of dark colored rosinate.

The practice of the invention seen in the foregoing illustrations is capable of many modifications without departing from the essential principle of retaining dark rosinates saturating a solvent for rosinates so that white rosinates do not dissolve. Among such variations that will be mentioned below are routine modifications which may be introduced during commercial adaptation, the introduction of water, changes in the solvent, and changes in the alkali.

Practical considerations and utilities may lead to many modifications of the way in which the process is practiced. For example, the carbonate may be added first to the petroleum, followed by the rosin, without the operation of the invention being affected.

In cases where there is a tendency of dark rosinate to precipitate before filtration, further rosin may be added at the end of the reaction in order to hold this dark rosinate in solution.

The petroleum solution can be fortified with fresh rosin, and re-used a number of times, before the dark material need be separated from it and the petroleum recovered by distillation. The better the grade of rosin employed, the more times the petroleum can be recycled.

When dark rosinate shows a tendency to come out during the filtration, and the product is to be washed, the initial washings can be made with a warm to hot solution of kerosene containing a little rosin; then with warm petroleum; next with petroleum at room temperature; and then finally with low-boiling petroleum. The final solvent is

of course readily separated from the rosinate by warming in a vacuum, or by otherwise allowing it to evaporate.

Mixtures of solvents can be used.

Dried sodium rosinate may be added to a solution of rosin in petroleum as mentioned in the first illustration of the theory of the process. Also partially neutralized rosinate can be used.

These and many other variations can be used without departing from the fundamental nature of the process, these being merely adaptations such as persons skilled in chemical processes would apply at convenience.

The invention can be practiced with alkali in aqueous solution, if the proportions of rosin, ros-

inate, and solvent at the end of the process are such as to permit retention of the dark rosinate in solution. But aside from possibly aiding rapidity of neutralization of the rosin acids, and a more complete utilization of the alkali, inclusion of water contributes little of value, and the introduced water must later be removed.

As the quantity of water is increased the difficulty of its removal becomes greater. More solvent must be used, so that evaporation of the hydrocarbon solvent will facilitate the removal of the water. The rosinate is very apt to form a gel, which makes stirring more and more difficult, and requires still more solvent to thin the mixture to a suitable consistency. The temperature must be raised higher and higher, in order to drive out the water, with result that above 180° C. the danger of cracking the rosin, or causing other undesirable changes, is increased. In the end the extra solvent must be distilled from the mixture, until the rosin concentration is suitable for holding the dark rosinates in solution while the white rosinate material separates. The use of much water makes it necessary to recirculate or add petroleum until at the end of the process the operator may well have used four, five, or even as much as ten times the amount of solvent necessary, all of which must be distilled from the reaction mixture with consequent danger of injuring the product.

The method above described for arriving at the preferred state employs anhydrous materials and adds more alkali than is necessary to neutralize the rosin, sometimes an excess of 50% or more, but this practice seems as good as if not better than one which, by introducing water, requires excessively large apparatus, distillation of much solvent, generally higher temperatures, additional expense, and also raises the danger of having the reaction mixture set to a gel, or if injuring the product by employing high temperature, any of which might nullify the commercial value. Excess of dry alkali, and vigorous stirring, are used

in the present process because precipitated rosinate tends to cling to the alkali bodies and so to obstruct progress of the reaction.

The rosin solvent to be employed should be a liquid immiscible with water and chemically inert to the rosin, rosinates and alkali concerned in the

expense and the incidental degradation of product involved when later steps have to be taken to eliminate introduced water. The table shows the invention practiced under conditions which are in the somewhat critical zone of concentration of rosin.

TABLE V  
WG rosin in kerosene with other alkali

| No. | Rosin,<br>g. | Alkali,<br>g.                      | Total<br>mix.,<br>cc. | Concen-<br>tration<br>of rosin<br>by weight<br>in solution,<br>percent | Ratio,<br>alkali to<br>rosin,<br>percent | Max.<br>temp.,<br>°C. | Time,<br>hrs. | Yield,<br>percent | Sodium<br>rosinate; color |
|-----|--------------|------------------------------------|-----------------------|------------------------------------------------------------------------|------------------------------------------|-----------------------|---------------|-------------------|---------------------------|
| 22  | 480          | NaOH 45                            | 1,750                 | 34                                                                     | 10                                       | 153                   | 2             | 49                | White.                    |
| 23  | 240          | NaOH 25                            | 1,750                 | 37                                                                     | 10.4                                     | 160                   | 1.5           | 55                | Shady white.              |
| 24  | 480          | K <sub>2</sub> CO <sub>3</sub> 112 | 1,750                 | 34                                                                     | 23.3                                     | 145                   | 2.5           | 50                | Snow white.               |

process, and preferably should be one whose boiling point is above the maximum temperature of reaction, except that for special purposes elsewhere explained the mixing in of a little having a lower boiling point is useful. For making the distinction between dark and light rosinates the liquid has to be one that dissolves rosin but does not dissolve rosinate except when it has unneutralized rosin in solution. All organic solvents are solvents for rosin, but the requirements as to boiling point and immiscibility with water render some of them unsuitable. The appropriate petroleum fractions, e. g. kerosene and ligroin, serve excellently, and other liquids also can serve.

Table IV illustrates this. In the summarized series of examples, item 20; each using 8 g. of WG rosin, the turpentine, xylene, and chlorobenzene gave products ranging between white and snow white, whose physical appearance was sometimes not as good for purposes of filtration as that from petroleum, but the product was found to be in general the same.

In Example 21, using 480 g. of WG rosin the solution in xylene was heated to 99° C. after which 80 g. of sodium carbonate was added, the temperature rising gradually with stirring for one and three-quarters hours to 136° C., and the mixture was then filtered at once, while hot. The product was a white sodium rosinate.

In all of these cases the water which forms as a result of the reaction should be removed promptly, even by raising the reaction temperature to the boiling point of the solvent, if necessary, in order to prevent gelling.

Metallic sodium may be used as the alkali. For example, 25 g. of this metal is added at 115° C. over a period of three minutes, with stirring, to a solution of 480 g. of rosin in enough kerosene to make a total volume of 1750 cc. A very vigorous exothermic reaction occurs, temperature rising within five minutes to 140° C. After stirring at this temperature for one hour the mixture, allowed to cool to about 80° C. and filtered, yields sodium rosinate, snow white save for some specks of sodium. The expense of metallic sodium, and the danger of small quantities of the metal being occluded in the product, with dangerous effect when the rosinate is dissolved in water, retard the practical use of this form of practicing the invention.

This invention can be practiced on a wide variety of resinous materials having the general composition of the acids in rosin, viz. C<sub>20</sub>H<sub>30</sub>O<sub>2</sub> or thereabouts. The showing of favorable conditions hereinbefore made indicates that probably the best material is crude gum, as obtained from the tree—after being filtered to remove dirt and other extraneous matter—because in this crude state the material has not undergone the heat treatment customary for removing its turpentine, and therefore it has fewer color bodies present. Besides the examples previously given (Table II) of the use of this material in very concentrated solution, Table VI shows the practice of the invention in the region of operation which is more critical because the rosin is less concentrated. Crude gum, 588 g., containing

TABLE IV  
WG rosin in other solvents, with Na<sub>2</sub>CO<sub>3</sub>

| No. | Rosin,<br>g. | Na <sub>2</sub> CO <sub>3</sub> ,<br>g. | Total<br>mix.,<br>cc. | Ratio<br>alkali to<br>rosin,<br>per cent | Max.<br>temp.,<br>°C. | Time,<br>hrs. | Solvent                                                  | Sodium rosinate; color |
|-----|--------------|-----------------------------------------|-----------------------|------------------------------------------|-----------------------|---------------|----------------------------------------------------------|------------------------|
| 20  | 8            | 2                                       | 16                    | 12.5                                     | 150                   | 3             | Summarized series: xylene turpentine chloro-<br>benzene. | Snow white to white.   |
| 21  | 480          | 80                                      | 1,750                 | 16.6                                     | 136                   | 1.75          | Xylene                                                   | White.                 |

Table V shows the invention practiced with use of other alkalis. Caustic soda, for example, can be employed, although more expensive and more troublesome to handle. The reaction produces more water than when anhydrous sodium carbonate is used, for eliminating which a quantity of petroleum solvent boiling within the range from 100° to 160° C. was used with the kerosene. In each case the better practice introduces no water as such, and so avoids both the substantial

about 80% rosin and 20% turpentine, being 470 g. net of rosin, was dissolved in enough kerosene to make the volume be approximately 1750 cc. At 100° C. sodium carbonate, 85 g., was added, with stirring, and the temperature was raised gradually to 149° C. over a period of two and a quarter hours. The mixture was then filtered at 100° C., and washed, first with kerosene to remove mother liquor, and then with low-boiling petroleum to remove the kerosene. A beautifully

snow white product was obtained, the yield being 57%.

TABLE VI  
*Pale crude gum, which would produce WG rosin, and Na<sub>2</sub>CO<sub>3</sub> in kerosene*

| No. | Rosin by calculation, g. | Na <sub>2</sub> CO <sub>3</sub> , g. | Total mix, cc. | Concentration of rosin by weight in solution, percent | Ratio alkali to rosin, percent | Max. temp., °C. | Time, hrs. | Yield, percent | Sodium rosinate, color |
|-----|--------------------------|--------------------------------------|----------------|-------------------------------------------------------|--------------------------------|-----------------|------------|----------------|------------------------|
| 25  | 470                      | 85                                   | 1,750          | 33                                                    | 18.7                           | 149             | 2.2        | 57             | Snow white.            |
| 26  | 473                      | 130                                  | 1,750          | 33                                                    | 21.9                           | 190             | 3.0        | 70             | White.                 |
| 27  | 474                      | 120                                  | 1,750          | 33                                                    | 20.0                           | 188             | 2.3        | 66             | Do.                    |

Wood rosin, particularly the FF grade, is generally considered to be an inferior variety by reason of the large number and variety of color bodies present. Illustrations have been given in Table I of the use of these materials in high percent rosin solution. Table VII shows the application in a zone of more critical concentration. In all cases colored rosinates are removed, but the degree of whiteness is not as high as that given in Table I. In the case of FF wood rosin, after the rosin was dissolved in the kerosene, the solution was preliminarily filtered to remove the considerable quantity of matter insoluble in the kerosene, and than was treated as described. Successful results from very poor grades of rosin are partly affected by the insolubility of its extraneous matter in the solvent. As the concentration of rosin in the kerosene solution diminishes, more of this insoluble matter is found precipitated with the precipitation of rosinate.

TABLE VII  
*Wood rosin and Na<sub>2</sub>CO<sub>3</sub> in kerosene*

| No. | Rosin, g.   | Na <sub>2</sub> CO <sub>3</sub> , g. | Total mix, cc. | Concentration of rosin by weight in solution, percent | Ratio alkali to rosin, percent | Max. temp., °C. | Time, hrs. | Yield, percent | Sodium rosinate, color |
|-----|-------------|--------------------------------------|----------------|-------------------------------------------------------|--------------------------------|-----------------|------------|----------------|------------------------|
| 28  | FF wood 400 | 60                                   | 1,750          | 28                                                    | 12.5                           | 160             | 2.5        | 22             | Gray white.            |
| 29  | FF wood 303 | 65                                   | 1,750          | 22                                                    | 21.1                           | 160             | 2.5        | 43             | Light brown.           |
| 30  | K wood 537  | 80                                   | 1,750          | 37                                                    | 14.9                           | 142             | 1.5        | 34             | Snow white.            |

Abietic acid is the product of isomerization of the rosin acids under acid influence. The commercial product contains the dark rosin acids which make this material degrading when used in soap. Practice of the present invention on this product led to isolation of a white sodium abietate: Commercial abietic acid, 120 g., was dissolved in enough kerosene to make a volume of 285 cc. The mixture was then heated to 125° C. at which temperature 36 g. of anhydrous sodium carbonate was added. The mixture was mechanically stirred, as in the other cases, was heated to 149° C. during the course of an hour, and was maintained at between 149° C. and 152° C. for one hour longer. By the usual cooling, filtration and washing, snow white sodium abietate was recovered.

These numerous illustrations show the wide range of conditions under which the invention can be practiced and the great variety of starting materials which can be employed. From any of such the process of the invention can produce a rosinate that is white, isolated from all dark rosinates as well as from all resenes, esters and all other dark or unsaponifiable substances.

The white rosinate thus isolated can be described as the sodium or potassium salts of rosin acids which, when in solid state, have the dis-

tinguishing visual characteristic that the solid is white.

Having the detergent properties that characterize all rosinates it can be mixed with the salts of other fatty acids in the manufacture of soap, and its standing as a rosinate which has properties distinctive from those of other rosinates as above indicated constitutes the product an improvement in rosin soaps in which the rosin present cooperates benignly with the other ingredients, without the depreciating effect heretofore experienced.

In the appended claims, the term "inert," applied to the liquid solvent, indicates only its lack of reactivity with the substances that may be present, i. e. alkali, water, unneutralized rosin acids, rosinates, resenes, esters and whatever other products remain after rosin has been treated with a base; "rosin," unless context indicates otherwise, signifies a body whose acid component is unneutralized rosin acids; "concentration of rosin" in the solution means the ratio

of rosin to the total of rosin plus its solvent, by weight; "rosinate" refers to the heterogeneous mixture of rosinates produced by neutralization of the various acids that may be present in rosin, and includes the rosinate of any one of those acids in a pure form of the acid, e. g. abietic acid; and white rosinate is considered to be "isolated" when it is separated from other rosinates, and substances contained in or derived from rosin, as rosin is known in commerce, regardless that non-resinous substances, e. g. alkali or petroleum, may be mixed with it or adhering to it.

I claim as my invention:

1. A process for dividing white alkali metal rosinate from dark alkali metal rosinate characterized by the step of subjecting a heterogeneous mixture of alkali metal rosinates to the solvent action of a solution of rosin in kerosene, in which the rosin-kerosene solution holds in solution all dark rosinate of the mixture, by its affinity for dark rosinate in preference to white rosinate; white rosinate that was in the said mixture and not taken into the rosin-kerosene solution being left in solid form.

2. The art of separating white alkali metal rosinate from other alkali metal rosinates, characterized by the step that all of the said rosinates

are immersed in a solution of rosin in kerosene which solution has a saturation point for dissolving rosinates that is high enough to permit of all dark rosinates present being dissolved and low enough to leave some white rosinate undissolved; the rosin-kerosene solution holding dark rosinate in solution in preference to white rosinate; and the said saturation point being fixed by having the concentration of rosin in the rosin-kerosene solution commensurate with that required for dissolving the quantity of dark rosinate which is present.

3. A process for dividing white alkali metal rosinate from dark alkali metal rosinate characterized by the step of subjecting a heterogeneous mixture of alkali metal rosinates to the solvent action of a solution of rosin in a petroleum solvent, in which the rosin-petroleum solution holds in solution all dark rosinate of the mixture, by its affinity for dark rosinate in preference to white rosinate, while some white rosinate of the said mixture remains undissolved.

4. A process for dividing white alkali metal rosinate from dark alkali metal rosinate characterized by the step of subjecting a heterogeneous mixture of alkali metal rosinates to the solvent action of a solution of rosin in a liquid organic solvent, which said organic solvent by itself alone is not a solvent for rosinate, is chemically inert to rosin, to rosinate, and to water, and is immiscible with water, in which step the rosin-organic solvent solution holds in solution all dark rosinate of the mixture, by its affinity for dark rosinate in preference to white rosinate; and some white rosinate of the mixture stands undissolved.

5. A process for segregating alkali metal white rosinate from other rosinates in a mixture of rosinates by holding the mixture immersed in a solution of rosin in a liquid organic solvent, which said organic solvent by itself alone is not a solvent for rosinate and is chemically inert to rosin and to rosinate and to water and is immiscible with water, in which said solution a concentration of rosin is maintained such that the rosin-organic

solvent solution has a dissolving capacity for rosinates, determined by the quantity of rosin present, which capacity is commensurate with a dissolving of all dark rosinate that is present but not all white rosinate that is present, by preferential affinity of the rosin-organic solvent solution to dissolve dark rosinate before it dissolves white rosinate; followed by filtering out the undissolved matter.

10 6. A process for producing alkali metal white rosinate apart from other rosinates; following a reaction in which a salt of an alkali metal is reacted with rosin that is in solution in a liquid organic solvent, which said organic solvent by itself alone is not a solvent for rosinate and is chemically inert to rosin and to rosinate and to water and is immiscible with water, thereby producing heterogeneous rosinates, in which process, after the said reaction, the concentration of rosin and the saturation point of the rosin-organic solvent solution for dissolving rosinates, determined by that concentration of rosin, are made commensurate with a dissolving of all dark but not all white rosinate that is present, determinable by sampling and testing, by preferential affinity of the rosin-organic solvent solution to dissolve dark rosinate before it dissolves white rosinate.

20 7. A process for producing alkali metal white rosinate apart from other rosinates, as in claim 6, characterized in that during the said reaction and process the concentration of rosin varies from an initial high proportion, approximating equality with the weight of the organic solvent, down to a final lower proportion sufficient to hold dissolved all dark rosinate that is present after the reaction but not sufficient to dissolve all white rosinate then present; fluidity of the mix during reaction being maintained by heating and stirring.

25 8. A process for producing alkali metal white rosinate apart from other rosinates as in claim 6, in which, during the reaction, the liquid body in which the reaction is occurring is maintained free from water.

AVERY A. MORTON.